

## UNITED STATES PATENT OFFICE.

LOUIS F. CLARK, OF JERSEY CITY, NEW JERSEY.

## TREATMENT OF LEAD MINERALS.

No Drawing.

Application filed April 23, 1924. Serial No. 708,330.

*To all whom it may concern:*

Be it known that I, LOUIS F. CLARK, a citizen of the United States, and resident of Jersey City, New Jersey, have invented certain new and useful Improvements in the Treatment of Lead Minerals, of which the following is a specification.

My invention aims to provide a process by which lead minerals can be made susceptible to concentration by the flotation method. Not all valuable minerals are amenable to flotation concentration. Generally only such as are called sulphides respond to such treatment. The other minerals, or such as may be called "oxides" because oxygen rather than sulphur is an important part of their composition, must first be given a preliminary treatment to make them recoverable in a flotation concentrate.

Minerals of lead are especially apt to fall under the above classification of sulphides and oxides. The sulphides will float and the oxides not. I have found, however, that when the oxides are given a preliminary coating of an organic substance, they too become floatable. The following description will show how such a substance of organic nature may be applied to the particles of lead mineral. The operations are performed in a pulp, that is, a mixture of finely ground ore and water. In such a condition the lead minerals may be considered as individual small particles whose surfaces may be modified by other substances dissolved in the water of the pulp. These reactions may be effected in various ways, as follows:

(a) Treatment of a pulp containing an oxide of lead, for example, lead carbonate, with an alkali bichromate, for example,  $Na_2Cr_2O_7$ , in a neutral or slightly acid solution to form a coating of lead chromate. This may advantageously be done in a solution having copper sulphate dissolved together with the alkali bichromate, or by a solution of copper bichromate itself. The equation for this last will indicate the net result of any such combination,—



It should be noted that this type of reaction is hastened by being a reciprocal precipitation, that is, both the new products formed on the surface of the lead minerals are relatively insoluble substances except in stronger acid solutions. This operation

should be conducted with small and insufficient amounts of the dissolved salts present to react with the total weight of lead carbonate in the portion of ore treated so as to merely coat the lead minerals and almost completely consume the dissolved salts.

After the above coating has been formed the lead minerals have a surface which is capable of oxidizing and so precipitating many organic substances which may now be introduced into the solution. A particularly important reagent for this purpose is aniline oil or an acid salt of aniline. This may be dissolved in the water of the pulp and a final coating of the organic oxidation product known as aniline black formed on the surface of the lead minerals. Other substances may serve the same purpose, for example, linseed oil, turpentine, pine oil, etc.

The function of the copper salt mentioned together with the alkali bichromate is to catalyze the final oxidation reaction between the chromate and the organic substance, for example, aniline, dissolved. There may, however, be sufficient copper mineral naturally associated with the lead carbonate so that its use in the operation may be omitted. On the other hand, the use of the copper salt in the operation may be delayed until the aniline is also dissolved. In this case a coating of lead chromate only would be formed. This would then be modified by a solution of say aniline and copper sulphate dissolved together to form the final organic resin coating on the lead minerals.

The above describes reactions which take place best in neutral or slightly acid solutions. The following procedure in alkaline solution may be more desirable with some ores, for example where lead carbonate occurs with limestone.

(b) Treatment of a pulp with bleaching lime, calcium hypochlorite, dissolved in the water of the pulp together with aniline oil. In this case in alkaline solution the lead minerals act catalytically at their surface to complete the oxidation of the aniline from the blue solution formed when it is dissolved with calcium hypochlorite, probably by incipient precipitation of lead dioxide. The net result is however the formation of the insoluble organic resin coating on the surface of the lead minerals. Other oxidizing agents in alkaline solution may be similarly employed, for example, hydrogen

peroxide, ferri-cyanides, and other organic substances, such as linseed oil, pine oil, etc. In all cases the lead minerals act catalytically at their surface to oxidize and precipitate the organic substance dissolved.

(c) Finally a more forceful procedure may be adopted for some ores. This may consist in applying a preliminary coating of a copper compound on the surface of the lead minerals in neutral or alkaline solution as previously mentioned. Equations illustrating these conditions follow:



15 This is a reciprocal precipitation from a solution of copper sulphate by the solid grains of lead carbonate to form the two new and relatively insoluble substances, lead sulphate and copper carbonate.



This is a deposition of copper cyanide from its solution with alkali cyanide by consumption of the solvent itself on the surface of the lead minerals. It gives the same effect of reciprocal precipitation but in alkaline solution. These equations should be considered as examples of the type of reaction involved. The same results may be attained by other salts of copper dissolved.

After this preliminary coating with a copper compound has been accomplished, then the procedure given in my application No. 35 671,392 may be applied and in substantially the manner as therein set forth for the treatment of naturally occurring oxidized copper minerals. This procedure consists in applying to a pulp of the treated ore acetylene and other oxidizable organic substances, which facilitate the reduction of the cupric minerals, so as to apply to the particles thereof a coating which facilitates their subsequent flotation.

45 The above describes methods whereby

precipitates may be first formed on the surface of the oxide minerals of lead, such precipitates being in turn capable of oxidizing and so precipitating certain organic substances which may be now brought in contact with the modified lead minerals by being dissolved in the liquid of the pulp.

Though I have described with great particularity of detail certain embodiments of my invention, yet it is not to be understood therefrom that the invention is restricted to the particular embodiments disclosed. Various modifications may be made in the particular steps and in the order thereof and in the substitution of equivalent materials by those skilled in the art without departing from the invention as defined in the following claims.

What I claim is:

1. The method of treating ores containing lead minerals which consists in forming on the particles of such minerals a superficial film of lead chromate and treating the same with an organic substance to oxidize the latter and precipitate the oxidation products on the particles.

2. The process of claim 1 in which the superficial film contains copper carbonate as well as lead chromate.

3. The method of treating ores containing lead minerals which consists in subjecting the particles to the action of lead chromate and copper sulphate in a solution of an organic substance adapted to be oxidized so that the oxidation products are precipitated on the particles.

4. The method of treating ores containing lead minerals which consists in coating the particles preliminarily with a copper compound and then applying a coating containing cuprous acetylid.

In witness whereof, I have hereunto signed my name.

LOUIS F. CLARK.